

## UNITED STATES PATENT OFFICE

GEORGE A. RICHTER, OF BERLIN, NEW HAMPSHIRE, ASSIGNOR TO BROWN COMPANY,  
OF BERLIN, NEW HAMPSHIRE, A CORPORATION OF MAINE

## PAPERMAKING COMPOSITION

No Drawing.

Application filed May 22, 1928. Serial No. 279,849.

In the papermaking industry, a large number of the manufacturers depend upon pulp mills for all or part of their supply of raw material. This is particularly true in the 5 branch of the industry handling the manufacture of high grade bond, ledger and writing papers. The pulp mills sometimes supply these paper manufacturers with pulp in bulk form, e. g., in a wet, pressed condition, or 10 in the form of bales of comparatively thick sheets or laps of relatively dry pulp known in the trade as "drier sheet". Shipment of pulp in this latter form is sometimes considered preferable, for not only does it reduce freight charges, but the pulp is better 15 preserved during shipment and storage.

At the paper mill, the pulp is partially hydrated or gelatinized before it is run off on the papermaking machines. Thus, the pulp 20 is charged into beater engines along with sufficient water to ensure its circulation, and is broken up or disintegrated whereupon it is hydrated or gelatinized by the operation of the engines prior to formation into paper. 25 To produce paper of the desired characteristics, beating must be carried on until the pulp has been gelatinized to a certain slowness value which has been found to result in paper having such characteristics.

It is quite evident that papermakers prefer 30 as raw materials pulps which acquire a certain slowness value in a comparatively short time of beating, for if the pulp employed is difficultly hydratable, the papermaker must expend more energy and time in beating to 35 reach this slowness value, thus increasing beating costs and reducing the beater output of the mill. On the other hand, pulps of an easily hydratable character are usually inferior 40 in certain other papermaking characteristics to pulps of a more difficultly hydratable character. When pulp is difficultly hydratable, the fibers of such pulp are reduced in length by the longer beating treatment 45 necessary in arriving at the slowness value desired, to a much greater extent than more easily hydratable pulp, so that it is an inevitable result that using satisfactory pulps having different hydratabilities but having 50 the same fiber length and beating to the same

slowness value, the tear resistance of paper made from the more difficultly hydratable pulp will be less than that of the more easily hydratable pulp.

There are some pulping or pulp-treating processes which yield pulps having certain highly desirable characteristics, but which at the same time are difficultly hydratable. For instance, when wood pulp is refined to high alpha cellulose content and then 55 bleached, it acquires certain very desirable characteristics, such as high whiteness, softness and absorbency, high fiber length, and excellent ageing qualities, in these and other respects being comparable to high grade rag 60 fiber. Such refined pulp is, however, much more difficult to hydrate to a given slowness value than the original pulp, for instance sulphite pulp, in this respect also being comparable to high grade new rags. This disadvantage of difficult hydratability inherent 65 in many refined wood pulps, is accentuated when such pulp is marketed in the form of drier sheets, as pulp shipped in a dry condition hydrates less readily than when shipped 70 in a wet condition.

In my application Serial No. 144,180, filed October 25, 1926, I have described a method of treating a difficultly hydratable pulp, such as refined wood pulp, to produce a product which may be hydrated or gelatinized to a given slowness value as readily as pulps of the character of sulphite. As described in that application, this is accomplished by preparing a product, such as a drier sheet, consisting of a homogeneous blend of an un-beaten pulp of a difficultly hydratable character, with pulp which has been hydrated or gelatinized, the gelatinized pulp preferably being present in subordinate proportion, so 80 that when the blended product is beaten to papermaking slowness and formed into paper, the paper will possess maximum tear resistance, most of the fiber being beaten for a comparatively short period and thus 85 preserved in length. The optimum procedure is to mix or blend about 5% to 10% of highly gelatinized pulp with about 90% to 95% of the un-beaten fiber, as this mixture or blend 90 may be formed into drier sheets which, when 100

subjected to beater action, hydrate to paper-making slowness quite readily, the hydrated or beaten stock being composed of fibers of high average length, so that paper made therefrom is of high tear resistance. More specifically, the gelatinized pulp is prepared from unbeaten pulp similar to the unbeaten pulp with which the gelatinized pulp is thereafter blended.

10 According to the present invention, the pulp employed as the source of the gelatinized cellulose used in the blended pulp is an easily hydratable pulp of high potential Mullen strength, short fibered pulps such as 15 those obtained from birch, for instance, being highly suitable for this purpose. Preferably also, such easily hydratable pulp is one containing a relatively high percentage of pentosans, especially when ratty, hard papers 20 of optimum Mullen strength, maximum tear resistance and fold endurance are desired. The present invention thus makes possible the conditioning of a difficultly hydratable pulp with a minimum expenditure of energy 25 and using short-fibered pulps which are relatively inexpensive. Apparently the pentosans in the hydrated or gelatinized pulp serve to bond together the fibers of the paper, augmenting the bonding effected by the gelatinized cellulose, and so increasing Mullen strength. Inasmuch as the characteristic of 30 folding endurance is associated with the bonding together of the fibers or Mullen strength, an increase in Mullen strength is 35 accompanied by an increase in folding endurance, so that paper made from the pulp blend of the present invention has very high Mullen strength, folding endurance and tear 40 resistance.

40 The present invention may be applied in the production of papers having various characteristics. For example, if a hard, ratty, high grade paper is desired, the pulp blend may consist of a preponderant 45 portion of a high alpha cellulose wood fiber of comparatively poor hydratability and a subordinate proportion of a gelatinized, easily hydratable pulp of relatively high 50 pentosan content. In certain types of pulp, the characteristics of high pentosan content and easy hydratability usually go hand in hand, so that various pulps are available for the desired purpose. Thus, one may employ 55 as the easily hydratable pulp the short fibered pulp produced from wood of the character of birch, as such pulp, even when liberated by chemical processes of digestion, e. g., the sulphite process, has a relatively 60 high pentosan content, usually being above 65 6%. One may also employ other pulps, such as spruce sulphite pulp, which usually has a pentosan content of about 3.5% to 4.5%. If, on the other hand, paper having high 70 softness and flexibility is desired, the pulp 75 employed as the source of the gelatinized

cellulose is preferably a refined wood pulp which hydrates quite readily. Usually, pulps of the latter character have a comparatively high pentosan content, but even when quite high in pentosans, if they are blended 70 with refined wood fiber which is low in pentosans, the blend results in papers of comparatively high softness and flexibility.

An example of procedure which may be followed in producing a blended product having the characteristics desired for the manufacture of high grade papers may be substantially as follows. A refined, unbeaten wood pulp of high average fiber length and low pentosan content, which hydrates with 75 difficulty, is selected as the major portion of the raw material, because of its rag-like qualities and the excellent characteristics of 80 papers made therefrom. With the refined, 85 unbeaten pulp is mixed or blended a subordinate proportion of gelatinized pulp which hydrates readily. The gelatinized pulp is 90 preferably prepared in beaters of the stone-roll type, such as employed in the glassine paper industry, as beaters of this general 95 type yield better gels and may be operated more economically for this kind of work than the usual paper mill beaters. Preferably, the stock is cooled, while being gelatinized, as described and claimed in patent application Serial No. 224,427, filed October 6, 1927, as this makes possible more economical 100 operation and the production of high grade 105 gels. The mixing or blending of the gel with the unbeaten pulp may be conveniently 110 carried out in the usual beater engines, the 115 gel and unbeaten pulp preferably being 120 mixed at a consistency of about 3% to 3 1/2%, 125 as under these conditions a homogeneous 130 blending or mixing may be readily effected. 135 Preferably, the gelatinized portion is exceedingly 140 slow or well hydrated, as this permits 145 the use of a larger relative proportion of 150 unbeaten fiber of original length, and at the 155 same time yields a pulp blend having good 160 hydrating qualities. Thus, the addition to 165 and blending with the unbeaten, refined wood 170 pulp of a highly beaten birch sulphite pulp 175 which has been gelatinized to a slimy 180 consistency, yields a pulp blend which may be 185 formed into thick, dry sheets or laps of pulp, 190 which respond quite readily to hydration. 195 When a pulp blend of this character, containing, say, 5% to 15% birch pulp gel, is 200 hydrated or beaten to papermaking slowness, it 205 yields hard, ratty papers of high Mullen 210 strength, folding endurance and tear 215 resistance, these characteristics being desirable 220 in certain bond papers. The high Mullen 225 strength and folding endurance of the resulting 230 paper is attributable to the cementing together 235 of the fibers, not only by the gelatinized 240 cellulose but also by the pentosans furnished 245 by the sulphite pulp.

If, in any case, it is undesirable to blend 250

pulps such as birch or spruce sulphite pulp with a high alpha cellulose wood pulp, the pulp used as the source of the gelatinized cellulose may also be one of high alpha cellulose content, but produced under conditions rendering it easily hydratable. Using a pulp blend consisting of only refined wood pulp, papers of high softness, flexibility, and having maximum strength, tear resistance and 5 folding endurance may be produced, these characteristics being desirable in ledger, cover and coating papers. For instance, a refined wood pulp of relatively low pentosan content, say, 1% to 2.5%, which is difficultly 10 hydratable and which by itself yields papers of high tear resistance but not very high Mullen strength, may be blended with a gelatinized refined wood pulp which is of higher pentosan content, say, 2.5% to 6%, and which 15 by itself would yield harder, rattlier papers of much higher Mullen strength. Such higher pentosan-containing refined wood pulps may be of somewhat lower alpha cellulose content than refined wood pulps of lower 20 pentosan content and at the same time have highly desirable papermaking characteristics. For example, such higher pentosan-containing refined pulp may be produced as described in my U. S. Patent No. 1,635,637, issued 25 July 12, 1927, which describes the pulping of wood such as spruce in an acid sulphite liquor having combined and free  $\text{SO}_2$  contents of approximately equal proportions of 3% to 4% each to produce a pulp especially 30 high in pentosans, and the refining of such pulp by oxidative treatment, alkaline-digestion, and bleaching, to produce a refined product of comparatively high pentosan content. Preferably, the refined wood fiber of 35 higher pentosan content is beaten or hydrated to a markedly gelatinous or slimy condition, so that when, say about from 5% to 15% by weight of such gelatinized pulp is blended with the unbeaten, refined pulp of lower 40 pentosan content, a pulp blend results which upon beating hydrates readily to papermaking slowness. Such a blended product may 45 be formed into drier sheets and marketed in this desirable condition. When such sheets 50 are beaten at the paper mill to papermaking slowness and the beaten pulp run off into paper, the resulting paper has practically the same softness and flexibility as the paper producible from a refined wood pulp of difficult 55 hydratability and of low pentosan content, and possesses the advantage of higher Mullen strength.

While the present invention has been described as having particular utility in producing a pulp blend at the pulp mill and then marketing such a blend as in the form of drier sheet to be used as a raw material for papermaking, it should be understood that the present invention may also be applied in 60 papermaking where it is desired to produce

high grade papers using different types of pulps such as hereinbefore described as raw materials. In other words, assuming that a papermaker is supplied with unbeaten pulp such as refined wood pulp of a difficultly hydratable character, and birch or spruce sulphite pulp or a refined wood pulp of a more readily hydratable character, the procedure to be followed at the paper mill in accordance with the present invention is to hydrate or 70 gelatinize the more readily hydratable pulp, say, to a slimy consistency, then to blend a relatively small proportion, say, 5% to 15% of the gelatinized pulp with the unbeaten, more difficultly hydratable pulp, and to beat 75 the pulp blend to papermaking slowness. The beaten blend yields papers having high Mullen strength and tear resistance, the length of fiber having been preserved to a large degree. One could not produce papers having 80 such high tear resistance by beating a blend of the unbeaten pulps to the same degree of slowness, for by so doing the length of fiber of the blend as a whole would be reduced to 85 a greater degree, owing to the much longer 90 time of beating necessary. By beating a pulp blend wherein the major portion of fiber exists in unbeaten condition and a relatively small portion of which exists in a highly 95 gelatinized condition, the blend as a whole need be beaten for a much shorter period to 100 reach the desired papermaking slowness. In certain cases, sufficient gelatinized cellulose may be added to the unbeaten portion to eliminate a substantial beating of the blend. That 105 is to say, one may blend sufficient gelatinized cellulose into the unbeaten fiber to attain papermaking slowness without further beating except that necessary to effect a homogeneous 110 dissemination of the gelatinized cellulose throughout the unbeaten fiber. This results in papers in which most of the fibers exist in original length, such papers having exceptionally high tear resistance; particularly when the unbeaten portion is composed of 115 fibers of high fiber length such as a refined wood fiber.

While I have dealt with certain specific instances in which my invention may be applied to produce products having certain 115 characteristics, other applications of my invention will be evident to those skilled in the art without departing from the spirit or scope of invention as set forth in the appended claims.

#### What I claim is:

1. A papermaking composition containing at least two different kinds of pre-liberated, chemical pulps, one of said pulps being substantially unbeaten and of a difficultly hydratable character and the other being highly beaten and of an easily hydratable character.
2. A papermaking composition containing at least two different kinds of pre-liberated chemical wood pulps, one of said pulps being 125
3. A papermaking composition containing at least two different kinds of pre-liberated chemical wood pulps, one of said pulps being 130

substantially unbeaten and of a difficultly hydratable character and the other being beater-gelatinized and of an easily hydratable character, said unbeaten pulp preponderating in amount.

- 5 3. A papermaking composition containing at least two different kinds of pre-liberated chemical wood pulps, one of said pulps being a substantially unbeaten pulp having a pentosan content of less than 2.5% and the other being a beater-gelatinized pulp having a pentosan content greater than 2.5%.
- 10 4. A papermaking composition in the form of a "drier sheet" containing at least two different kinds of pre-liberated chemical wood pulps, one of said pulps being a substantially unbeaten refined pulp having a pentosan content of less than 2.5% and the other being a beater-gelatinized pulp having a pentosan content greater than 2.5%.
- 15 5. A papermaking composition in the form of a "drier sheet" containing at least two different kinds of pre-liberated chemical wood pulps, one of said pulps being a substantially unbeaten refined pulp having a pentosan content less than 2.5% and the other being a beater-gelatinized pulp having a pentosan content greater than 2.5%, said gelatinized pulp amounting to about 5% to 15% by
- 20 weight of the composition.

In testimony whereof I have affixed my signature.

GEORGE A. RICHTER.

35

40

45

50

55

60

65